

[54] ELECTRICAL INSULATION OIL

[75] Inventors: **Jiro Ogura; Ikuo Seki; Kiyotaka Sato**, all of Hitachi; **Masaaki Takahashi; Akira Ito**, both of Tokyo; **Yuriko Igarashi**, Mitaka, all of Japan

[73] Assignee: **Kureha Kagaku Kogyo Kabushiki Kaisha**, Tokyo, Japan

[22] Filed: Sept. 30, 1974

[21] Appl. No.: 510,224

[30] Foreign Application Priority Data

Oct. 4, 1973 Japan ..... 48-111869  
Nov. 15, 1973 Japan ..... 48-127669

[52] U.S. Cl. .... 252/63.7; 174/110 S; 252/63; 252/78

[51] Int. Cl.<sup>2</sup> ..... H01B 3/18  
[58] Field of Search ..... 252/63.7, 63, 78; 174/110 S

[56] References Cited

UNITED STATES PATENTS

2,340,644 2/1944 Clark ..... 252/63.2

FOREIGN PATENTS OR APPLICATIONS

538,411 8/1941 United Kingdom ..... 252/64

Primary Examiner—John D. Welsh  
Attorney, Agent, or Firm—Lane, Aitken, Dunner & Ziems

[57]

ABSTRACT

An electric insulating oil having excellent electrical insulation properties is obtained by incorporating in silicone oil at least one member selected from the group consisting of alkyl fluoranthenes of the generic formula



and alkyl pyrenes of the generic formula



wherein, R denotes an alkyl group having from one to four carbon atoms and x denotes an integer having a value of from 1 to 4, and when x is an integer of 2 or more, R may be the same or different.

3 Claims, No Drawings

## ELECTRICAL INSULATION OIL

## FIELD OF THE INVENTION

This invention relates to an electric insulating oil of the type used, in oil-immersed electric apparatus such as, for example, oil-immersed power cables and transformers.

## BACKGROUND OF THE INVENTION

10

The necessity for using a nonflammable oil having high thermal resistivity as an electric insulating oil for use in oil-immersed electric apparatus has become widely recognized. To meet this need, silicone oil has come to take the place of mineral oil which has previously served as an electric insulating oil.

Silicone oil is superior to mineral oil in terms of thermal resistivity and nonflammability but is inferior to mineral oil in dielectric breakdown voltage strength as shown in the following table. For this reason, the silicone oil does not, of itself, a fully satisfactory electric insulating oil.

|                        | Viscosity<br>(C.S.)<br>at 30°C | Dielectric<br>breakdown<br>voltage<br>strength<br>(KV) | 1.52<br>mm in<br>oil layer<br>thickness | 25 |
|------------------------|--------------------------------|--------------------------------------------------------|-----------------------------------------|----|
| Dimethyl polysiloxane* | 10                             | 26                                                     |                                         |    |
| Mineral oil**          | 10                             | 50                                                     |                                         |    |

\* KF-96-10, made by The Shin-Etsu Chemical Industry Co., Ltd.

\*\* Insulating oil No. 2, prescribed in JIS C-2320.

In order for silicone oil to be used effectively as an electric insulating oil, therefore, it is desirable that the silicone oil be improved in terms of dielectric breakdown voltage strength.

## SUMMARY OF THE INVENTION

It is, therefore, an object of the present invention to provide an electric insulating oil having excellent electric insulation by improving the dielectric breakdown voltage strength of the silicone oil without impairing its inherent properties of outstanding thermal resistivity and nonflammability.

Other objects of this invention will become apparent from the following description.

It has now been discovered that when at least one compound selected from the group consisting of specific alkyl fluoranthenes and specific alkyl pyrenes is incorporated into the silicone oil, the resultant mixture possesses high dielectric breakdown voltage strength and therefore serves quite satisfactorily as an electric insulating oil.

The present invention adds to the silicone oil at least one member selected from the group consisting of alkyl fluoranthenes of the generic formula



and alkyl pyrenes of the generic formula



wherein, R denotes an alkyl group having from one to four carbon atoms and x denotes an integer having a value of from 1 to 4, and when x is an integer of 2 or more, R may be same or different.

## DETAILED DESCRIPTION OF THE INVENTION

As previously noted, alkyl fluoranthenes which are used in the present invention are those represented by the generic formula:



30 wherein, R denotes an alkyl group having from one to four carbon atoms and x denotes an integer having a value of from 1 to 4, and when x is an integer of 2 or more, R may be same or different.

As is clear from the structural formula, these alkyl fluoranthenes have at least one alkyl group selected from the group consisting of methyl, ethyl, propyl and butyl attached at random positions in the fluoranthene nucleus. Such alkyl fluoranthenes can easily be obtained by isolation from coal tar and petroleum fractions which are rich in polycyclic aromatic hydrocarbons or by alkylating fluoranthenes with a lower olefin having up to four carbon atoms in the presence of a Friedel-Crafts type catalyst such as aluminum chloride or a solid acid catalyst such as silica-alumina. Generally, an alkyl fluoranthene has many isomers. For use in the present invention, a selected alkyl fluoranthene need not be in single isomeric form but may be in the form of a mixture of isomers.

The alkyl pyrenes which are used in the present invention are those represented by the generic formula:



wherein, R denotes an alkyl group having from one to four carbon atoms and x denotes an integer having a value of from 1 to 4, and when x is an integer of 2 or more, R may be same or different. From the structural formula, it is evident that these alkyl pyrenes have at least one alkyl group selected from the group consisting of methyl, ethyl, propyl and butyl attached at random po-

sitions in the pyrene nucleus. Such alkyl pyrenes can easily be obtained by isolation from coal tar fractions and petroleum tar which are rich in polycyclic aromatic hydrocarbons or by alkylating pyrenes with a lower olefin having up to four carbon atoms in the presence of a Friedel-Crafts type catalyst such as aluminum chloride or a solid acid catalyst such as silica-alumina. Generally, an alkyl purene has many isomers. For use in the present invention, a selected alkyl pyrene need not be in a single isomeric form but may be used in the form of a mixture of isomers.

As previously noted, the present invention incorporates into the silicone oil of at least one compound selected from the group consisting of alkyl fluoranthenes and alkyl pyrenes of the types described above. The

compound will not homogeneously mix with the silicone oil, almost regardless of the particular kind of silicone oil used.

The present invention will be described more specifically by the following description of the preferred embodiments.

#### EXAMPLE 1

Various alkyl fluoranthenes and alkyl pyrenes were added, individually and in the form of mixtures, in the percentages (%) shown in Table 1 to dimethyl polysiloxane (KF-96-10 made by The Shin-Etsu Chemical Industry Co., Ltd.) and the resultant mixtures were tested for dielectric breakdown strength. The results are shown in Table 1.

TABLE 1

| Name of additive    | Boiling point (°C) | Dielectric breakdown voltage strength (KV/1.5 mm of oil width) |       |       |                            |       |       |       |       |       |        |                               |
|---------------------|--------------------|----------------------------------------------------------------|-------|-------|----------------------------|-------|-------|-------|-------|-------|--------|-------------------------------|
|                     |                    | (0)                                                            | (0.1) | (0.2) | Amount added (% by weight) | (0.5) | (1.0) | (1.5) | (2.5) | (5.0) | (10.0) | (11.0)                        |
| Methyl pyrene       | 390-410            | 26.3                                                           | 31.0  | 37.3  | 47.0                       | 49.5  | 48.0  | 35.3  | 34.7  | 30.0  | 26.8   |                               |
| Ethyl pyrene        | 400-420            | 26.3                                                           | 30.5  | 37.5  | 47.3                       | 49.5  | 43.2  | 35.6  | 35.0  | 30.6  | 28.6   |                               |
| Butyl pyrene        | 420-460            | 26.3                                                           | 31.0  | 37.0  | 46.1                       | 48.3  | 42.5  | 37.0  | 34.9  | 31.5  | 27.3   |                               |
| Propyl pyrene       | 410-430            | 26.3                                                           | 30.4  | 36.5  | 45.2                       | 49.1  | 48.5  | 37.4  | 35.8  | 32.3  | 28.0   | Dielectric breakdown strength |
| Methyl fluoranthene | 380-440            | 26.3                                                           | 30.8  | 37.0  | 47.1                       | 49.0  | 47.5  | 35.5  | 34.0  | 29.7  | 27.3   |                               |
| Ethyl fluoranthene  | 390-410            | 26.3                                                           | 30.3  | 38.2  | 46.7                       | 48.5  | 40.7  | 38.2  | 35.5  | 32.0  | 28.2   |                               |
| Butyl fluoranthene  | 410-450            | 26.3                                                           | 29.8  | 37.5  | 45.5                       | 43.6  | 42.4  | 37.0  | 36.2  | 31.0  | 26.3   |                               |
| Propyl fluoranthene | 400-420            | 26.3                                                           | 30.2  | 38.1  | 46.0                       | 46.3  | 40.5  | 36.6  | 35.1  | 30.1  | 26.8   |                               |
| Mixture 1           | 390-520            | 26.3                                                           | 30.6  | 37.0  | 46.3                       | 40.5  | 41.3  | 35.9  | 35.8  | 31.5  | 26.5   |                               |
| Mixture 2           | 410-450            | 26.3                                                           | 30.0  | 37.0  | 45.5                       | 45.8  | 46.0  | 37.0  | 35.5  | 30.3  | 27.0   |                               |
| Mixture 3           | 400-500            | 26.3                                                           | 31.0  | 38.0  | 46.3                       | 42.6  | 42.0  | 36.5  | 36.4  | 30.6  | 27.2   |                               |
| Mixture 4           | 400-495            | 26.3                                                           | 30.3  | 37.3  | 45.2                       | 45.2  | 43.3  | 37.0  | 36.0  | 31.2  | 28.1   |                               |

  

| (Note)             | Mixture 1 |       | Mixture 2     |                     | Mixture 3 |        | Mixture 4     |                     |
|--------------------|-----------|-------|---------------|---------------------|-----------|--------|---------------|---------------------|
|                    | Pyrene    | 5 wt% | Propyl pyrene | Propyl fluoranthene | 50 wt%    | 50 wt% | Propyl pyrene | Propyl fluoranthene |
| Monopropyl pyrene  | 50 "      |       |               |                     |           |        |               |                     |
| Dipropyl pyrene    | 30 "      |       |               |                     |           |        |               |                     |
| Tripropyl pyrene   | 10 "      |       |               |                     |           |        |               |                     |
| Tetrapropyl pyrene | 5 "       |       |               |                     |           |        |               |                     |

amount of such compound added to the silicone oil should preferably fall in the range of from 0.1 to 10% by weight based on the silicone oil. If the amount is less than the lower limit 0.1% by weight, the compound fails to provide any appreciable improvement in the dielectric breakdown voltage strength. If, on the other hand, the amount added exceeds the upper limit 10% by weight, then the resultant mixture exhibits a degree of dielectric breakdown voltage strength inferior to that obtained by mixtures containing the compound in the range of from 0.1 to 10% by weight and the com-

45

#### EXAMPLE 2

Dimethyl polysiloxane (KF-96-10 made by The Shin-Etsu Chemical Industry Co., Ltd.) and mixtures obtained by adding various alkyl fluoranthenes and alkyl pyrenes, individually and in the form of mixtures, in a fixed weight percentage of 0.5% as shown in Table 2 were tested for dielectric properties (dielectric loss tangent and dielectric constant), thermal resistivity (stability against oxidation) and non-flammability (flash point). The results are shown in Table 2.

TABLE 2

| Name of additive    | Property |       | Dielectric loss tangent tan δ (%) |      | Dielectric constant |                    | Specific volume resistivity, $\rho$ (Ω cm) |                    | Stability(*) against oxidation | Flash(**) poing (°C) |
|---------------------|----------|-------|-----------------------------------|------|---------------------|--------------------|--------------------------------------------|--------------------|--------------------------------|----------------------|
|                     | 30°C     | 80°C  | 30°C                              | 80°C | 30°C                | 80°C               | 30°C                                       | 80°C               |                                |                      |
| None added          | 0.003    | 0.003 | 2.64                              | 2.45 | $3 \times 10^{16}$  | $1 \times 10^{16}$ | $1 \times 10^{16}$                         | $1 \times 10^{16}$ | 0.004                          | 154                  |
| Methyl pyrene       | 0.004    | 0.004 | 2.65                              | 2.46 | $2 \times 10^{16}$  | $1 \times 10^{16}$ | $1 \times 10^{16}$                         | $1 \times 10^{16}$ | 0.004                          | 153                  |
| Ethyl pyrene        | 0.004    | 0.005 | 2.66                              | 2.46 | $2 \times 10^{16}$  | $1 \times 10^{16}$ | $1 \times 10^{16}$                         | $1 \times 10^{16}$ | 0.004                          | 154                  |
| Butyl pyrene        | 0.005    | 0.005 | 2.68                              | 2.45 | $2 \times 10^{16}$  | $1 \times 10^{16}$ | $1 \times 10^{16}$                         | $1 \times 10^{16}$ | 0.005                          | 153                  |
| Propyl pyrene       | 0.005    | 0.004 | 2.64                              | 2.47 | $2 \times 10^{16}$  | $1 \times 10^{16}$ | $1 \times 10^{16}$                         | $1 \times 10^{16}$ | 0.005                          | 152                  |
| Methyl fluoranthene | 0.004    | 0.005 | 2.65                              | 2.47 | $2 \times 10^{16}$  | $1 \times 10^{16}$ | $1 \times 10^{16}$                         | $1 \times 10^{16}$ | 0.005                          | 153                  |
| Ethyl fluoranthene  | 0.005    | 0.005 | 2.68                              | 2.47 | $3 \times 10^{16}$  | $1 \times 10^{16}$ | $1 \times 10^{16}$                         | $1 \times 10^{16}$ | 0.005                          | 154                  |
| Butyl fluoranthene  | 0.004    | 0.005 | 2.67                              | 2.45 | $3 \times 10^{16}$  | $1 \times 10^{16}$ | $1 \times 10^{16}$                         | $1 \times 10^{16}$ | 0.004                          | 155                  |
| Propyl fluoranthene | 0.004    | 0.005 | 2.64                              | 2.48 | $2 \times 10^{16}$  | $1 \times 10^{16}$ | $1 \times 10^{16}$                         | $1 \times 10^{16}$ | 0.004                          | 156                  |
| Mixture 1           | 0.003    | 0.003 | 2.65                              | 2.47 | $2 \times 10^{16}$  | $1 \times 10^{16}$ | $1 \times 10^{16}$                         | $1 \times 10^{16}$ | 0.004                          | 155                  |
| Mixture 2           | 0.005    | 0.004 | 2.65                              | 2.47 | $2 \times 10^{16}$  | $1 \times 10^{16}$ | $1 \times 10^{16}$                         | $1 \times 10^{16}$ | 0.006                          | 154                  |
| Mixture 3           | 0.004    | 0.004 | 2.64                              | 2.46 | $2 \times 10^{16}$  | $1 \times 10^{16}$ | $1 \times 10^{16}$                         | $1 \times 10^{16}$ | 0.006                          | 155                  |

TABLE 2-continued

| Name of additive | Property |       | Dielectric constant |      | Specific volume resistivity, $\rho$ ( $\Omega$ cm) |                    | Stability(*) against oxidation | Flash(**) point (°C) |
|------------------|----------|-------|---------------------|------|----------------------------------------------------|--------------------|--------------------------------|----------------------|
|                  | 30°C     | 80°C  | 30°C                | 80°C | 30°C                                               | 80°C               |                                |                      |
| Mixture 4        | 0.005    | 0.005 | 2.64                | 2.45 | $3 \times 10^{16}$                                 | $1 \times 10^{16}$ | 0.006                          | 154                  |

(Note 1)

| Mixture 1          |    |     | Mixture 2           |    |     |
|--------------------|----|-----|---------------------|----|-----|
| Pyrene             | 5  | wt% | Propyl pyrene       | 50 | wt% |
| Monopropyl pyrene  | 50 | "   | Propyl fluoranthene | 50 | "   |
| Dipropyl pyrene    | 30 | "   |                     |    |     |
| Tripropyl pyrene   | 10 | "   |                     |    |     |
| Tetrapropyl pyrene | 5  | "   |                     |    |     |

  

| Mixture 3     |    |     | Mixture 4           |    |     |
|---------------|----|-----|---------------------|----|-----|
| Propyl pyrene | 50 | wt% | Propyl fluoranthene | 50 | wt% |
| Ethyl pyrene  | 50 | "   | Ethyl fluoranthene  | 50 | "   |

(Note 2)

(\*) Stability against oxidation —This value is in terms of dielectric loss tangent (%) which was measured after having heating a given sample at 100°C continuously in air for four days.

(\*\*) Flash point —measured by the Pensky-Martens method prescribed in JIS K-2265.

It is clear from the preceding two working examples that the additives of the present invention provide the silicone oil with improved dielectric breakdown voltage strength without impairing the outstanding dielectric properties, thermal resistivity and nonflammability inherent to silicone oils.

Since the electric insulating oil of the present invention possesses the highly desirable properties described above, it is especially useful for insulation of high-voltage electric apparatus. It may also be combined with a plastic material to form composite insulating material, having utility as insulation for high-voltage oil-filled power cables.

What is claimed is:

1. An electric insulating oil comprising a silicone oil and 0.1–10.0% by weight of at least one additive selected from the group consisting of alkyl fluoranthenes of the general formula



and alkyl pyrenes of the general formula



wherein, R denotes an alkyl group having from 1 to 4 carbon atoms and x is an integer of from 1 to 4, and when x is an integer of 2 or more, R may be same or different.

2. The electric insulating oil of claim 1, wherein said alkyl fluoranthene is present in the form of a mixture of isomers.

3. The electric insulating oil of claim 1, wherein said alkyl pyrene is present in the form of a mixture of isomers.

\* \* \* \* \*